

No. 627,229.

J. O. FOSTER.  
MANIFOLDING SHEET.  
(Application filed Mar. 9, 1896.)

Patented June 20, 1899.



Witnesses

Char A. Smith  
J. Staub.

Inventor

John O. Foster  
John O. Foster  
J. W. Darrell & Son  
atty

# UNITED STATES PATENT OFFICE.

JOHN O. FOSTER, OF NEWARK, NEW JERSEY.

## MANIFOLDING-SHEET.

SPECIFICATION forming part of Letters Patent No. 627,229, dated June 20, 1899.  
Application filed March 9, 1899. Serial No. 708,325. (No specimens.)

To all whom it may concern:

Be it known that I, JOHN O. FOSTER, a citizen of the United States, residing at Newark, in the county of Essex and State of New Jersey, have invented an Improvement in Transfer-Sheets for Manifold, or Duplicate Writing or Printing, of which the following is a specification.

The object of the present invention is to dispense entirely with separate sheets and to coat the back of one sheet with a material that is transferred to the prepared surface of the next sheet in order that the first sheet may be written upon by a pencil or otherwise and form the original and the second sheet is a duplicate of the writing of the first, thereby dispensing with any intermediate sheet. I prepare the back of the first sheet and the surface of the second sheet so that there is an offset from the back of the first sheet to the surface of the second sheet, and the materials preferred by me, as hereinafter described, are such as to be substantially waterproof, and if the transfer-writing should become obscure through the presence of moisture it is restored to sharpness when the material is dried, and by making use of three, four, or more sheets, the back of one being coated with the transfer material and the adjacent surface of the other being coated with the receiving material, any desired number of copies can be duplicated and it is only necessary to tear off or remove these copies in succession.

While the present improvement is especially adapted to railroad and express work, it is not in any way limited, but can be employed for ordinary correspondence and can be used upon type-writers or printed upon, a duplicate or duplicates being produced by the impression upon the original, whether that impression be made by the types in the type-writer, by a pencil, pen, or otherwise.

In carrying out this present invention I place on the back of the original sheet white or light-colored clay, chalk, or similar material in a pulverulent condition and caused to adhere by suitable material, and upon the surface of the second sheet a contrasting color is employed and with a surfacing material that is slightly adhesive, so that the pressure upon the original sheet causes the magnesia,

clay, or other material to be transferred to the surface of the second sheet and to adhere to the same firmly, and the materials preferably employed by me, as hereinafter set forth, are not easily influenced by moisture. Hence the transfer becomes permanent and reliable, and where the second sheet has a backing similar to the first sheet a transfer can be simultaneously made therefrom to a third sheet having a prepared surface, and so on any desired number of transfers or manifold writing or printing can be simultaneously effected.

In the drawing I have illustrated a number of the sheets, and it is to be understood that the surface of sheet 1 is to be written upon or printed and that the back surface *a* of this first sheet is prepared with the transfer material and the front surface *b* of sheet 2 is prepared with the receiving material, and where more than one copy is to be made simultaneously the back surface *c* of the second sheet 2 is also prepared with transfer material similar to the back of sheet 1, and the surface *d* of the third sheet 3 is to be prepared with the receiving material and the surface *e* with the transfer material, and so on any desired number of sheets can be prepared and employed, and while it is true that the first sheet 1 might have a receiving-surface, so that all the sheets would be alike, I find it generally advantageous to make the first sheet 1 with a plain surface adapted to a pencil or pen or to be printed upon by type-writing or otherwise.

The transfer material may be composed of magnesia, clay, bronze-powder, or other material having more or less color and in a pulverulent condition. I find that china-clay is well adapted to this purpose, and the same is mixed with an adhesive substance. I have found that about two per cent. of glue and about three per cent. of shellac form a very good material for causing the light-colored pulverulent material to adhere together and to the back of the sheet, and caoutchouc or india-rubber, resin, or similar material may be added, and it is generally preferable to dissolve the shellac in ammonia and to mix the materials in a hot condition to a consistency of cream and then to apply such material to the backs of the sheets, and when the same

becomes dry it is adapted to the transfer-work before mentioned.

If it should be found that the light-colored pulverulent material rubs off upon the hands or smears, the proportion of adhesive material can be increased. If, on the other hand, it is too hard for easy transfer, the proportion of glue or other adhesive material may be lessened, and this transfer material may be applied with a brush or by a roller to the backs of the sheets.

The receiving-surfaces of the sheets are to be of a contrasting color to the transfer material. They may be black, brown, purple, red, blue, green, or other color, and the film or receiving-coating is advantageously composed, in addition to the coloring-matter, of resin, stearic acid, paraffin, Japan wax, or resin and beeswax, such materials being melted together and applied to the surfaces of the sheets. I find that paraffin in three parts, caoutchouc in the comminuted form, rubber cement in one part, and resin and stearic acid in about equal parts produce a good receiving-surface when applied hot to the surface of the paper and laid on evenly by rollers, brushes, or otherwise. Tissue-paper can be easily prepared as the receiving-film, care being taken to fill in fine perforations and to coat the entire surface of the paper with uniformity.

If the sheet with the receiving upper surface or film is also to be used as a transfer-sheet, as illustrated at 2, 3, and 4, the backs of such sheets are coated with the light-colored transfer material before mentioned.

When the first sheet is written or printed upon, the pressure at the lines of the printing, writing, or drawing causes the transfer material from the back of one sheet to adhere firmly to the adjacent surface of the next sheet, and when the sheets are separated the transfer or manifold writing can be easily read by the contrast between the material that is caused to adhere from the back of the first sheet upon the surface of the second sheet, and so on, where there are more than two sheets made use of, and it will be found that the light-colored coating upon the back of one sheet is substantially removed upon the lines of pressure to the adhering surface of the receiving-film and the transfer is not liable to become smeared or obliterated, and if water is applied or an effort made to wash off the record sufficient of the light-colored transfer material will be found adhering to the receiving-surface to become legible after such surface dries.

I remark that a small per cent. of bichromate of potash or tannic acid mixed into the solution for the transfer-surface renders the glue insoluble, so that the same cannot easily be washed off, and that the adhesive character of the glue is not materially interfered with.

65 I do not limit myself to the ingredients

herein described, as the same may be varied according to the circumstances of use.

I claim as my invention—

1. For manifold-writing, a sheet prepared with a light-colored transfer material upon the back, and a second sheet prepared with a darker-colored receiving-surface, that is sufficiently adhesive to receive and hold the material transferred from the back of the first sheet to the surface of the second sheet by pressure upon the surface of the first sheet by a pen, pencil, types, or otherwise, substantially as set forth.

2. For manifold-writing, a sheet of paper adapted to being written upon and having a coating upon the back of pulverulent light-colored material caused to adhere by a mixture of adhesive material, in combination with a second sheet having a surface of adhesive material to which the material from the back of the first is caused to adhere by the pressure in writing, printing or drawing, substantially as set forth.

3. A sheet of paper for manifold-writing having upon the back light-colored material in a pulverulent condition with an adhesive material mixed therewith, and adapted to adhere to a second sheet at the places where there is pressure from writing or printing upon the first sheet, substantially as specified.

4. A transfer-sheet for manifold-writing having on the back a coating of clay in a pulverulent condition and an adhesive material, such as glue, mixed therewith and bichromate of potassium, tannic acid or similar material to render such glue substantially waterproof, substantially as set forth.

5. A manifold-sheet coated on both surfaces, the one surface having an adhesive material, such as a wax or resinous material and the other surface having a coating of pulverulent material in a contrasting color and adhesive material to hold the coating upon the back of the sheet, substantially as set forth.

6. For manifold-writing, a sheet of paper adapted to being written upon and having a coating upon the back of pulverulent material and adhesive material, in combination with a second sheet having a surface of adhesive material of a color contrasting to the color of the material that is transferred from the back of the first sheet by the pressure in writing, printing or drawing, substantially as set forth.

7. A manifold-sheet coated on the face with an adhesive material such as a wax or resinous material and on the back with pulverulent and adhesive materials, substantially as specified.

Signed by me this 6th day of March, 1899.

JOHN O. FOSTER.

Witnesses:

GEO. T. PINCKNEY,  
S. T. HAVILAND.